

[72] Inventor **Davis M. Batson**  
Baton Rouge, La.  
[21] Appl. No. **619,888**  
[22] Filed **Feb. 24, 1967**  
[45] Patented **Jan. 11, 1972**  
[73] Assignee **Ethyl Corporation**  
New York, N.Y.

[54] **INCENDIARY COMPOSITIONS**  
4 Claims, No Drawings

[52] U.S. Cl. .... **149/87,**  
149/109, 44/7  
[51] Int. Cl. .... **C06b 15/00**  
[50] Field of Search. .... **149/87,**  
109; 44/7

[56] **References Cited**  
UNITED STATES PATENTS  
2,765,329 10/1956 Lindsey ..... 149/87 X  
3,084,181 4/1963 D'Alelio ..... 149/109 X  
3,280,088 10/1966 D'Alelio ..... 149/109 X

*Primary Examiner*—Carl D. Quarforth  
*Assistant Examiner*—Stephen J. Lechert, Jr.  
*Attorney*—Donald L. Johnson

**ABSTRACT:** Self-igniting, gellike incendiary compositions are prepared by thickening aluminum alkyls and/or aluminum alkyl hydrides with an alkyl branched butadiene polymer. Additionally, the incendiary may contain diluents which are compatible with aluminum alkyls such as hydrocarbons, finely divided metals, and certain organometallic compounds. These incendiaries may be used in firebombs, fire rockets, flame throwers, aerial flares, and other military applications.

## INCENDIARY COMPOSITIONS

## BACKGROUND OF THE INVENTION

This invention relates to incendiary compositions and to methods of dispensing them to produce an effective conflagration.

Incendiary compositions such as contained in firebombs, fire rockets, or ejected from flame throwers, now generally in use, are ignited by means of a fuse, a spark, or some other external mechanism. The ignition process may be commenced when the incendiary is propelled or released from the source or the ignition mechanism may be actuated when the projectile strikes the target. While these ignition techniques have achieved a degree of success, they are subject to malfunction and the incendiary composition may not ignite and, thus, is totally ineffective.

Current incendiary compositions consist mainly of gelled or thickened gasoline. While this material is usually quite flammable, it must be independently ignited and often does not burn completely. Upon striking the target, only that portion remaining in the area of ignition will burn. Because of its relatively high volatility, the unburned gasoline will quickly vaporize and, thus, preclude any possibility of future ignition. Moreover, the burning of these compositions is not very intense and may be extinguished or otherwise rendered ineffective for the purpose intended.

Another shortcoming with current incendiary compositions, and particularly those ejected from equipment such as a flame thrower, is the extremely short range. Even when ejected under high pressure and, therefore, at high velocities, the incendiary composition, ignited as it leaves the flame thrower, is completely burned within a relatively short range from the source. Thus, the use of this type equipment is limited to extremely short range applications.

## SUMMARY OF THE INVENTION

A self-igniting incendiary composition, having a gellike consistency, is obtained by thickening from about 65 to about 98 weight percent of an aluminum compound having the formula



wherein R is an alkyl group and x is an integer from one to three, with from about 2 to about 10 weight percent of cis-polyisoprene gelling agent. The composition may also contain from zero to about 20 weight percent of a diluent.

## DESCRIPTION OF THE INVENTION

The incendiary compositions of this invention are self-igniting incendiaries containing varying percentages of aluminum compounds thickened with a polyisoprene. More specifically, the aluminum compounds contemplated are the alkyl and alkyl hydride aluminums, hereinafter referred to simply as aluminum alkyls. The compounds have the formula:



$H_{3-x}$  where R is an alkyl group containing from one to four carbon atoms, and x is an integer ranging from one to three. In a preferred embodiment, R is a lower alkyl group containing up to three carbon atoms and x is equal to two or three. These materials are more reactive than the higher alkyls and, thus, assure maximum effectiveness. The most preferred embodiment comprises a composition wherein the aluminum alkyl component consists of from 90 to 100 percent triethylaluminum and from zero to 10 percent diethylaluminum hydride. This composition is preferred because it is of intermediate reactivity, volatility, and stability and is relatively economical to manufacture.

The compositions of this invention are incendiaries of extremely high reliability. They possess properties which produce a more intense and effective conflagration than heretofore possible. Furthermore, these incendiaries are self-

igniting, burn with an intense flame, have low volatility, and are extremely difficult to extinguish. After discharging, the incendiaries of this invention, as a rule, do not ignite immediately but only after some delay, thereby increasing the effective range of instrumentalities such as flame throwers. Upon ignition, they provide an intense, widespread and effective conflagration.

The compounds which are useful in the incendiary compositions of this invention include trimethylaluminum, 10 dimethylaluminum hydride, methylaluminum dihydride, triethylaluminum, diethylaluminum hydride, ethylaluminum dihydride, tripropylaluminum, dipropylaluminum hydride, propylaluminum dihydride, tributylaluminum, dibutylaluminum hydride, butylaluminum dihydride, triisobutylaluminum, 15 diisobutylaluminum hydride, isobutylaluminum dihydride. The higher alkyl derivatives including the amyl and hexyl compounds and aromatic derivatives such as the phenyl, tolyl, xylyl, etc. compounds of aluminum can also be used, especially as diluents and to impart certain characteristics to the aluminum alkyl mixture.

The polyisoprene employed in this invention may be prepared by any of the known methods such as fluid-bed, fixed-bed, and solution polymerization processes. The 25 catalysts employed in any of the processes mentioned is not critical. Examples of the catalysts used in fluid-bed polymerization processes are alfin catalysts which are complexes formed by a sodium salt of methyl-n-alkyl carbinol, e.g., sodium isopropoxide, and a sodium adduct with an olefin 30 such as propylene, e.g., allylsodium; alkali metals such as lithium, sodium, potassium, cesium and rubidium; organolithium compounds including alkyl, allyl, aralkyl, and alkaryl compounds such as n-butyllithium, n-amyllithium, isoamyllithium, phenyl, tolyl, and benzyllithium as well as polyllithium 35 hydrocarbons such as hexamethylenedithilithium and 1,5-naphthalenedilithium; Ziegler-type catalysts, especially those prepared from vanadium or titanium trichlorides, in conjunction with aluminum triethyl, as well as catalysts prepared from vanadium oxychloride or chromylchloride and aluminum triethyl or zinc diethyl. Similar Ziegler catalysts can be also employed in solution polymerization processes.

The molecular weight of the polymer is not critical. However, it should be of such molecular weight and such viscosity that it would permit the polymer to be at least partially soluble 45 in lower alkylaluminum compounds. Preferably, the polymer should be only partially soluble at ambient temperature and considerably more soluble at elevated temperatures, especially around 100° C.

Although polyisoprene is preferable in this invention, other 50 branched chain butadienes may also be employed. Examples of such additional polymers are those obtained from monomers such as 3-ethyl-1,3-butadiene, 3-propyl-1,3-butadiene, 3-butyl-1,3-butadiene, 2,3-dimethyl-1,3-butadiene, 55 2,3-diethyl-1,3-butadiene, 2,3-dibutyl-1,3-butadiene, and the like.

The most preferred polyisoprene employed in this invention is cis-polyisoprene which has a high cis-1,4 content. A specific example of this type of polyisoprene is Natsyn-200. It is a beige colored solid polyisoprene elastomer manufactured by a solution polymerization process employing a stereospecific catalyst. The cis-1,4-content of the polymer is approximately 95 percent, and the molecular configuration duplicates that of natural rubber. The polymer contains a nonstaining, non-discoloring stabilizer. Although no molecular weight is given, the Mooney viscosity ML-4 at 212° F. is 80 to 100.

This invention provides thickened or gelled incendiary compositions. Such compositions comprise from about 65 to about 65 weight percent aluminum alkyls, from about 2 to about 10 weight percent of a thickening agent, and from 0 to about 25 weight percent of a diluent.

Another aspect of this invention provides a method of producing a conflagration which comprises dispersing a diluted or thickened incendiary composition as described 75 above in or over a target area.

The aluminum alkyls are ideally suited as incendiary materials, for upon contact with air, they spontaneously ignite and burn with an intense flame. Therefore, the igniting mechanism, which is required with prior art incendiaries, is eliminated. Concentrated aluminum alkyls also react with water to give a violent and sometimes explosive reaction. The compounds also react with other compounds containing active hydrogen such as alcohols, amines, organic and inorganic acids, and to some extent, with materials such as paper and cloth. Therefore, the application of the incendiary compositions of this invention is not restricted to an air media but can be used in a wide variety of applications with maximum reliability and effectiveness.

The thickened or gelled incendiary compositions generally adhere tenaciously to the intended target. Also, by the addition of the thickening agent and, if desired, a diluent, the ignition delay period of the aluminum alkyls may be altered so as to obtain the desired duration. Moreover, in applications such as a flame thrower, a thickened composition may be propelled over a long distance.

Depending upon the specific application, the incendiary compositions may be in different forms. The consistency of the mixture may vary from a mobile fluid to a highly thickened gel. The consistency is varied by including up to about 20 percent of the thickener and, if desired, a diluent. Amounts of the diluents and thickeners in much greater concentration than the above limit impairs the ignition properties of the incendiary compositions.

The addition of diluents to the thickened aluminum alkyls serves a variety of purposes. By selection of the proper diluent, an incendiary composition may be obtained that has optimum properties with respect to density, volatility, reactivity, ignition delay characteristics, etc., and in many cases provides a more economical mixture. Broadly, any material which is compatible and does not react with aluminum alkyls or the thickener may be used as a diluent. It is preferable that the material to be used as a diluent is itself capable of combustion when heated to its kindling temperature. The materials useable as diluents include hydrocarbons, finely divided metals, and organometallic compounds, preferably those not containing reactive functional groups, and not containing oxygen or reactive hydrogen. More specifically, petroleum derived hydrocarbons such as gasoline, kerosene, tar, asphalt, petroleum jelly, heavy lubricating oil, mineral oil, etc., are useable. Metals such as iron, magnesium, aluminum, zinc, boron, lithium, sodium, etc., in a finely divided state, or their organic compounds such as diethylzinc, tributyl borine, may be used. Other organometallic compounds may also be used, especially those containing a cyclomatic radical such as dicyclopentadienyl iron, methylcyclopentadienyl manganese tricarbonyl, dicyclopentadienyl manganese, etc. Other metallic compounds may be included in the compositions, especially sodium hydride, sodium aluminum hydride, sodium borohydride lithium borohydride, or any of the sodium alkali metal hydrides, aluminum hydrides, or borohydrides. These normally solid compounds are partially soluble in the aluminum alkyls. The higher alkyl and aromatic compounds of aluminum such as tripentylaluminum, trihexylaluminum, triphenylaluminum, etc., may also be included as diluents. These materials are much less reactive than the lower alkyls and, thus, may be employed to obtain a less reactive, more controllable incendiary composition.

The compositions of this invention are useable in a wide number of military applications. This invention provides "tailormade" thickened aluminum alkyls which are ideal for military incendiary use, specifically for antipersonnel or anti-material applications. The compositions may also be used in fire bombs, fire rockets, in the form of frangible capsules or spheres propelled from devices such as a compressed gas gun or mortar which could launch a package of such capsules. Aluminum alkyl compositions are also ideally suited as flame thrower fuels. The compositions of this invention are self-igniting, producing a higher flame temperature than normally

used materials such as gelled gasoline and, in addition, cause both chemical and thermal injuries to personnel. These compositions are also amenable to nonmilitary applications such as flares either of the stationary type or discharged from a hand pistol as aerial flares, etc.

An example of the incendiary bomb provided by this invention comprises a sheet-steel shell having a ballistic configuration tapering down to a forward nose section which is constructed of heavy steel to facilitate penetration into the intended target. The rear portion of the shell terminates in a tail assembly which includes an opening through which the shell is filled with the incendiary composition, and fins to stabilize the flight of the bomb and, thus, improve accuracy. Appropriate means such as a threaded plug are used to seal the opening after filling. The bomb may be jettisoned from an aircraft singly or it may be in a cluster from which individual bombs are released during the descent. The above-described incendiary bomb is designed to fracture due to its own momentum when it strikes the target, thereby releasing its content. Alternatively, the bomb may be equipped with any of the well-known types of bursting charges for fragmenting the bomb shell and thereby forcefully expelling the incendiary compositions. A fuse designed to function instantaneously upon impact or with a delayed action is incorporated into the nose section to ignite a small charge of explosive material such as gun powder also contained therein. The igniting mechanism may also be designed to fire while the bomb is in flight prior to striking target.

Many benefits accrue from the use of the incendiary compositions of this invention which were heretofore not obtainable. One important advantage is that the compositions are self-igniting when exposed to air. Accordingly, the independent ignition mechanism of current incendiaries is obviated, thereby precluding any failure of the ignition mechanism.

Another important advantage of this invention is that upon exposure to air, there is a certain delay period before self-ignition takes place. The ignition delay period varies with different aluminum alkyl compounds. For example, the ignition delay period for trimethylaluminum is much shorter than for a higher alkyl such as tributylaluminum. Moreover, the ignition delay period may be altered somewhat by altering the amounts of a polyisoprene thickening agent and of the diluent. Thus, a "tailormade" composition is available with various ignition delays periods. In this manner, the effective range of instrumentalities such as flame throwers can be increased, and only a part of the fuel will be burned before reaching the intended target.

Another advantage in using the incendiaries of this invention is that they are less volatile than currently used materials for this purpose. The aluminum alkyls will not evaporate as readily as gasoline and, thus, the material will burn on the surface of the target, thereby providing maximum effectiveness. The aluminum alkyls burn vigorously with an extremely hot flame and are, therefore, much more difficult to extinguish than conventional incendiaries. These incendiaries also burn with a cleaner flame, with a minimum of smoke, thereby making it difficult to locate and extinguish the flame.

The following examples illustrate the methods of preparing the compositions of this invention. All parts are by weight unless otherwise specified.

#### EXAMPLE 1

65 To a vessel placed in a nitrogen atmosphere were added 100 parts of triethylaluminum and 6 parts of cis-polyisoprene which was first cut in approximately  $\frac{1}{8}$ -inch cube-pieces. After heating the mixture to about 100° C., the contents were thoroughly mixed. The resulting incendiary composition had a consistency of medium thick gum and ignited immediately upon exposure to air.

70 A 1-milliliter sample of the above composition was burned on an asbestos board. A chromel-alumel thermocouple was inserted in the burning mass in the various parts of the flame. The maximum flame temperature was found to be 1,330° F.

Similar compositions are obtained when in the above example, a mixture of triethylaluminum and diethylaluminum hydride is employed in place of triethylaluminum.

## EXAMPLE 2

Following the procedure of example 1, 9 parts of cis-polyisoprene was mixed with 100 parts of triethylaluminum. An incendiary having the consistency of a uniform heavy gum was obtained. Upon exposure to air, the composition exhibited delayed ignition.

About 20 weight percent of mineral oil is added to the above composition. The resulting incendiary has a somewhat lighter consistency.

A substantially similar composition is obtained when 10 parts of cis-polyisoprene is employed.

## EXAMPLE 3

Following the procedure of example 1, two parts of cis-polyisoprene was mixed with 100 parts of triethylaluminum. The resulting incendiary had a consistency of light slush.

To the composition obtained in example 3 is added about 20 weight percent of a diluent such as powdered iron, sodium, and aluminum. The resulting incendiary has a vapor pressure lower than the incendiary without a diluent.

In addition to the above specific embodiments, many other applications of the compositions of this invention and articles of manufacture will be obvious to those skilled in the art. Besides other miscellaneous applications such as booby traps and clandestine devices, the compositions may be used in land mines, or rocket projectiles, and fire starters in general. These incendiary compositions may also be used for nonmilitary pur-

poses as, for example, in fire bombs or aerial spraying to start "backfires" in fighting forest fires.

The aluminum alkyls are well known compounds. Methods for their preparation can be found in any standard texts including "Organometallic Compounds," by G. E. Coates, 1960, John Wiley and Sons, Inc., New York, N. Y.; "Organic Chemistry" by P. Karrer, 1950, Elsiveier Publishing Company, New York, N. Y., etc.

Having fully defined the novel incendiary compositions of 10 this invention and the methods of using them, it is desired that this invention be limited only within the lawful scope of the appended claims.

I claim:

1. A thickened incendiary composition having a gellike consistency consisting essentially of from about 65 to about 98 weight percent of an aluminum compound having the formula



20 wherein R is an alkyl group and x is an integer ranging from one to three; and from about 2 to about 10 weight percent of cis-polyisoprene gelling agent and from zero to about 20 weight percent of a diluent.

25 2. The composition of claim 1 wherein said aluminum compound is triethylaluminum.

3. The composition of claim 1 wherein said aluminum compound is a mixture of triethylaluminum and diethylaluminum hydride.

30 4. The composition of claim 1 consisting essentially of 94 weight percent of triethylaluminum and 6 weight percent of cis-polyisoprene.

\* \* \* \* \*

35

40

45

50

55

60

65

70

75